

## UNITED STATES PATENT OFFICE

2,173,821

## METHOD OF MAKING A STIFFENED FABRIC

Bjorn Andersen, Maplewood, N. J., assignor to  
 Celluloid Corporation, a corporation of New  
 Jersey

No Drawing. Application May 5, 1936,  
 Serial No. 77,916

9 Claims. (Cl. 154—2)

This invention relates to the manufacture of stiffened articles and more particularly to the manufacture of box toes for shoes employing as the stiffening material a fabric impregnated with a derivative of cellulose.

An object of the invention is the economic and expeditious production of stiffened articles such as counters, box toes, inner soles and other parts of shoes and like objects. Another object of the invention is the production of stiffening material which more readily and more uniformly adheres to the surface and lining layers of the article in which the stiffening material is used. Other objects of the invention will appear from the following detailed description.

The manufacture of box toes or shoe stiffeners is generally carried out by precipitating a cellulose derivative in the form of fine particles in the interstices of a cloth or other sheet material. After the cloth has been impregnated with the cellulose derivative and allowed to dry, blanks of convenient shape and size are cut out by the shoe manufacturer. These blanks are then dipped for a very short time in a solvent bath, the strength of which is carefully regulated to impart the desired degree of gelatinization and pliability. For the purpose of describing this invention and in the appended claims this solvent bath will be referred to as the softening solution. While in this flaccid and swollen condition, the blanks are cemented or laminated between an inner cloth lining and the outside leather layer. The reinforced composite is then shaped over a wooden last to the contour of the shoe and the solvents allowed to volatilize, with the formation of a stiffened form.

I have discovered a unique method of insuring a very intimate and uniform adhesion between the stiffening material and the contacting layers. This method comprises adding to the solvent bath in which the blanks are dipped an agent, preferably a base such as ammonia, which dissolves or cuts into the usual finishes on the inner fabric lining and leather outer layer and/or otherwise causes the stiffening material to readily seize and adhere to said contacting layers. It is very important for efficient hand or mechanical operations that the stiffening sheet readily seize and adhere to the other layers. In most shoe factories one operator assembles the blanks, gives them a light rolling with a hand roller and tosses them into a basket or conveyor to be carried to the operator who applies them to the last. If the stiffening material does not adhere strongly to the lining and leather, they become separated

prior to reaching to the last. If the stiffening material does not readily seize onto the lining and leather, it greatly slows up production since it necessitates a longer and more strenuous pressing together of the layers. Where shoes having cut-out decorations are being formed, heavy pressing must be avoided as this causes the plastic material to be pushed into the cut-out portions. 5

In accordance with my invention, I employ, in the manufacture of stiffened articles containing a sheet material comprising a base sheet impregnated with a derivative of cellulose as the stiffening member, a softening solution which renders the stiffening member soft, adhesive and moldable. The softening solution comprises a solvent for the derivative of cellulose employed and an agent that cause the softened stiffening member to seize and adhere to other sheet material. The solvent may be any suitable reagent or mixture of reagents having a solvent action upon the derivative of cellulose, while the added agent may be any agent that causes the softened material to seize and adhere to other sheet material, such agents may be water, an organic acid or, more preferably, an inorganic basic compound 15 such as ammonia. 20

This invention is applicable to the formation of stiffened articles such as box toes, counters, inner soles, etc. of shoes, belts, supports, collars and like wearing apparel and also to industrial articles such as cases for technical instruments, sheaths for cutting instruments, caps for breeches of field artillery, etc. The outer layer, in most cases named above, will be leather while 35 the inner layer is of varying weights of muslin. However, this invention is not limited to such assemblies. For instance, any flexible or semi-flexible sheet material may be employed as either the lining layer or the outer layer. Examples of 40 suitable sheet materials for use as the lining or outer layers are leather, patent leather, imitation leather, fabrics of silk, cotton, wool, artificial fibres or filaments, felts, paper and the like. 30

The stiffening member or layer may be formed 45 of any suitable base material impregnated with a derivative of cellulose. The base material may be any suitable cloth formed from cotton fibers, silk, animal fibers, artificial fibres and filaments, etc. The base material may be impregnated with 50 any suitable derivative of cellulose in any suitable manner. Examples of suitable derivatives of cellulose are cellulose nitrate, cellulose acetate, cellulose nitro-acetate, cellulose formate, cellulose propionate or other esters of cellulose. Cel- 55

lulose ethers and the ether-esters of cellulose may also be employed such as cellulose aceto butyrate.

Blanks cut from the stiffening material are dipped for a very short time in a softening solution which renders them soft and hand moldable. When moistened with the softening solution, they are pressed between a cloth lining and a leather layer after which they are shaped on a last. Heretofore trouble has been experienced at this

10 point in the manufacture since the blanks failed to seize quickly and adhere to the other layers. For instance, when the softening solution is a low boiling solvent, there is formed, upon evaporation, a skin coating which is not adhesive. In 15 accordance with this invention, I form a softening solution which overcomes the difficulties arising from lack of adhesion in the stiffening material by adding to the softening solution an agent which produces an adhesive property in 20 the stiffening material. This agent is preferably an inorganic alkaline substance either soluble in the softening solution or at least in one component of the softening solution. Although sodium, potassium and other alkaline or alkaline

25 earth metal hydroxides may be employed, I prefer to employ, whenever possible, ammonium hydroxide owing to the volatile nature of the same. Organic base substances may also be employed, such as triethyl amine, triphenyl amine, triethanolamine, etc. These alkaline or basic substances are referred to in the claims as "alkalis." I have also found that good adhesive properties may be imparted to the stiffening material by adding, in place of the alkaline or basic substance, a concentrated organic acid to the softening solution. Examples of such organic acids are formic acid, glacial acetic acid, etc. I may also employ a small amount of water to effect the property of good adhesion.

35 40 The quantity of the agent, which produces an adhesive property in the stiffening material, added to the softening solution may vary from less than 0.5 to more than 5% based on the volume of the softening solution. The quantity employed for best results will depend upon the particular agent employed. When employing acetone as the softening solution and cellulose acetate or cellulose nitrate as the derivative of cellulose in the stiffening material the amount of ammonium hydroxide (commercial grade of about 28% NH<sub>3</sub>) required to produce good adhesive properties is from 0.5 to 5% by volume. The softening solutions containing ammonia, if allowed to stand until the characteristic odor of the ammonia has largely dissipated, are not impaired in softening and cementing qualities.

55 60 The softening solution may be formed of one or a mixture of low boiling solvents, with or without plasticizers and high boiling solvents for the particular derivative of cellulose employed in the stiffening material or sheet. Examples of suitable solvents for cellulose esters are acetone, methyl acetate, methyl cellosolve (mono methyl ether of ethylene glycol), cellosolve (mono ethyl ether of ethylene glycol), chloroform, ethylene dichloride, mixtures of ethyl or methyl alcohol and acetone, mixtures of ethylene dichloride and ethyl or methyl alcohol, etc. Examples of plasticizers that may be employed either in the derivative of cellulose impregnating material or in the softening solution are the aryl sulphonamides such as para ethyl toloul sulphonamide, the alkyl phthalates such as dimethyl phthalate, the di-alkyl tartrates such as dibutyl tartrate, the alkoxy esters of polybasic organic acids such as

diethoxy ethyl phthalate, the polybasic acid esters of the mono alkyl ethers of polyhydric alcohols, such as diethylene glycol ethyl ether ester of phthalic acid, the alkyl ester of phosphoric acid such as triethylglycol phosphate, the aryl esters of phosphoric acid such as tricresyl phosphate, the mixed alkyl and aryl phosphates such as ethylglycol diresyl phosphate, and camphor.

5 10 The drying time or period of stickiness of the stiffening material may be varied by adding to the softening solution higher boiling solvents. Examples of suitable higher boiling solvents for nitrocellulose and cellulose acetate are methyl cellosolve, methyl cellosolve acetate, diacetone alcohol, benzyl alcohol, beta, beta dichlorethyl ether.

15 Examples of softening solutions particularly applicable to cellulose acetate box toe material are:

*Example I*

|                                  | Parts by volume | 20 |
|----------------------------------|-----------------|----|
| Methyl acetate                   | 100             |    |
| $\beta\beta'$ dichlorethyl ether | 5               |    |
| Commercial ammonium hydroxide    | 4               |    |

*Example II*

|                                  | Parts by volume | 25 |
|----------------------------------|-----------------|----|
| Acetone                          | 100             |    |
| $\beta\beta'$ dichlorethyl ether | 10              |    |
| Methyl cellosolve acetate        | 10              |    |
| Commercial ammonium hydroxide    | 3               | 30 |

*Example III*

|                     | Parts by volume |    |
|---------------------|-----------------|----|
| Methyl cellosolve   | 80              |    |
| Diacetone alcohol   | 15              |    |
| Glacial acetic acid | 5               | 35 |

*Example IV*

|                           | Parts by volume |    |
|---------------------------|-----------------|----|
| Methyl acetate            | 50              |    |
| Diacetone alcohol         | 50              | 40 |
| Methyl cellosolve acetate | 100             |    |
| Benzyl alcohol            | 50              |    |
| Ammonium hydroxide        | 3               |    |

An example of a suitable softening solution for nitrocellulose box toe material is:

*Example V*

|                     | Parts by volume |    |
|---------------------|-----------------|----|
| Acetone             | 65              |    |
| Ethyl methyl ketone | 8               | 50 |
| Ethyl alcohol       | 8               |    |
| Amyl acetate        | 40              |    |
| Dimethyl phthalate  | 3               |    |
| Ammonium hydroxide  | 1               |    |

*Example VI*

|                   | Parts by volume |  |
|-------------------|-----------------|--|
| Methyl acetate    | 100             |  |
| Methyl cellosolve | 25              |  |
| Water             | 5               |  |

*Example VII*

|                           | Parts by volume |    |
|---------------------------|-----------------|----|
| Methyl acetate            | 100             |    |
| Methyl cellosolve         | 75              |    |
| Methyl cellosolve acetate | 75              | 65 |
| Water                     | 5               |    |

When high boiling solvents are added to the softening solution the amount of agent producing an adhesive property in the stiffening material may be reduced. In some formulas the quantity of alkaline or other agent may be reduced to below 0.5% by volume.

The addition of the alkaline agent to the softening solution not only gives to the treated material an adhesive property but also acts to

aid the softening solution to more readily and uniformly wet-out the material dipped in same.

It is understood that the foregoing detailed description is given merely by way of illustration and that many variations may be made therein without departing from the spirit of my invention.

Having described my invention, what I desire to secure by Letters Patent is:

- 10 1. A softening solution for use in rendering moldable a stiffening material containing a derivative of cellulose, comprising a low boiling solvent for the derivative of cellulose and an alkali which has a softening action on the material of the article to which the stiffening material is to be applied.
- 20 2. A softening solution for use in rendering moldable a stiffening material containing an ester of cellulose, comprising a low boiling solvent for the ester of cellulose and an alkali which has a softening action on the material of the article to which the stiffening material is to be applied.
- 25 3. A softening solution for use in rendering moldable a stiffening material containing a derivative of cellulose, comprising a low boiling solvent for the derivative of cellulose and aqua ammonia which has a softening action on the material of the article to which the stiffening material is to be applied.
- 30 4. A softening solution for use in rendering moldable a stiffening material containing an ester of cellulose, comprising a low boiling solvent for the ester of cellulose and aqua ammonia which has a softening action on the material of the article to which the stiffening material is to be applied.
- 35 5. In a method of stiffening toes of shoes and other articles by the use of a stiffening material containing a derivative of cellulose, the steps of applying to an article comprising an outer layer and the stiffening material a softening solution containing a solvent for the derivative of cellulose and from .05 to 5% by volume of an alkali which has a softening action on said outer layer, shaping the treated article and drying the same.

lose and an alkali which has a softening action on said outer layer, shaping the treated article and drying the same.

6. In a method of stiffening toes of shoes and other articles by the use of a stiffening material containing an ester of cellulose, the steps of applying to an article comprising an outer layer and the stiffening material a softening solution containing a solvent for the ester of cellulose and an alkali which has a softening action on said outer layer, shaping the treated article and drying the same.

7. In a method of stiffening toes of shoes and other articles by the use of a stiffening material containing a derivative of cellulose, the steps of applying to an article comprising an outer layer and the stiffening material a softening solution containing a solvent for the derivative of cellulose and a small amount of aqua ammonia which has a softening action on said outer layer, shaping the treated article and drying the same.

8. In a method of stiffening toes of shoes and other articles by the use of a stiffening material containing an ester of cellulose, the steps of applying to an article comprising an outer layer and the stiffening material a softening solution containing a solvent for the ester of cellulose and a small amount of aqua ammonia which has a softening action on said outer layer, shaping the treated article and drying the same.

9. In a method of stiffening toes of shoes and other articles by the use of a stiffening material containing a derivative of cellulose, the steps of applying to an article comprising an outer layer and the stiffening material a softening solution containing a solvent for the derivative of cellulose and from .05 to 5% by volume of an alkali which has a softening action on said outer layer, shaping the treated article and drying the same.

BJORN ANDERSEN.